

March 24, 1959

**TOSHIO HAYASAKA ET AL**  
**ACOUSTICAL TITANIUM DIAPHRAGM AND METHOD**  
**FOR HEAT TREATING SAME**

Filed May 3, 1956

2,879,193

2 Sheets-Sheet 1



INVENTORS  
TOSHIO HAYASAKA  
KENRO MASUZAWA  
SHOZO NAGAI

By *William D. Carothers*  
THEIR ATTORNEY

March 24, 1959

TOSHIO HAYASAKA ET AL  
ACOUSTICAL TITANIUM DIAPHRAGM AND METHOD  
FOR HEAT TREATING SAME

2,879,193

Filed May 3, 1956

2 Sheets-Sheet 2



INVENTORS  
TOSHIO HAYASAKA  
KENRO MASUZAWA  
SHOZO NAGAI

By: *William D. Casother*  
THEIR ATTORNEY

1

2,879,193

## ACOUSTICAL TITANIUM DIAPHRAGM AND METHOD FOR HEAT TREATING SAME

Toshio Hayasaka, Kenro Masuzawa, and Shozo Nagai, Tokyo, Japan, assignors to Nippon Telegraph & Telephone Public Corporation, Tokyo, Japan, a corporation of Japan

Application May 3, 1956, Serial No. 582,598

Claims priority, application Japan May 11, 1955

7 Claims. (Cl. 148—21.9)

This invention relates to a diaphragm for acoustic apparatus, and more particularly to a diaphragm made of titanium.

It is well known that duralumin is generally used as material for acoustic diaphragm. Compared with duralumin, titanium has substantially the same strength/density; however, it has a stronger resistance against corrosion; its drawability and formability are superior to those of duralumin; and its coefficient of thermal expansion is smaller. Therefore, the diaphragm made of titanium is considered excellent for acoustic apparatus of high quality, for example, standard apparatus for acoustic measurement. It must be noted, however, that, in case a diaphragm which is always under stress, such as a diaphragm for telephone receivers and a diaphragm for condenser microphones, is made of titanium, the efficiency of the apparatus varies gradually, due to deformation thereof caused by creep phenomenon of titanium, and therefore, the stability of efficiency cannot be expected.

The object of the present invention is to provide a titanium diaphragm for acoustic apparatus in which the efficiency is substantially invariable.

In order to accomplish the above object, the feature of the present invention is to make a diaphragm by forming a titanium sheet in a desired form, and thereafter applying heat treatment thereto, or to make a diaphragm by applying heat treatment to a titanium sheet at the state where tension is applied.

The results of the experiments made by the inventors revealed that a titanium diaphragm obtained by forced aging, which constitutes the characteristic of the invention, produces almost no diaphragm deformation to be caused by creep phenomenon, in case such diaphragm is used for telephone receivers or condenser microphones.

In the attached drawings,

Fig. 1 shows the variation of resonance frequency of a diaphragm for condenser microphones, by taking the lapse of time as abscissa.

Fig. 2 shows the pull which works to a diaphragm for telephone receivers, as function of air gap length.

Fig. 3 shows the deformation of a diaphragm for telephone receivers as function of the lapse of time, in case a load of 1,000 gr. w. is applied thereto.

To a diaphragm for condenser microphones, a stress of about 15 kg./mm.<sup>2</sup> is always working. Therefore, the diaphragm is gradually elongated and the stress working thereupon is decreased whereby the resonance frequency is lowered down, and as the result thereof, the efficiency of the microphone gradually increases. The resonance frequency of the diaphragm, which is formed with a titanium sheet, without forced aging, is lowered down, as shown by the curve I in Fig. 1, as time elapses. In view of the characteristic of the curve I, it is supposed that about one year's time is required for the diaphragm to stabilize, by ceasing to deform, and to be practically used. On the other hand, the variation of resonance frequency of a diaphragm to which heat treatment has been

2

applied for 6 hours at the temperature of 200° C. in the air, at the state where tension is worked after the formation of the titanium sheet, is as shown by the curve II in Fig. 1. In the course of the heat treatment, the resonance frequency is abruptly lowered down as shown by the dotted line B. However, after the heat treatment, the resonance frequency of the diaphragm is remarkably stabilized as shown by the curve d—e. The value of the resonance frequency shown by the part d—e in the curve

5 II is supposed to be almost equivalent to that of the resonance frequency, to be arrived at by a diaphragm, to which no heat treatment is made, after having been left to stand for decades.

It must be noted that, in a diaphragm for condenser microphones, no stabilized resonance frequency, as shown by the curve II in Fig. 1, can be attained, if tension is applied thereto after heat treatment.

To a diaphragm for telephone receivers, a pulling force is always working by permanent magnet. This pulling force is the function of air gap as shown in Fig. 2, which is about 300 gr. w. at working gap, and about 1000 gr. w. at zero gap. Therefore, the diaphragm for telephone receivers is deformed by the creep phenomenon due to the above pulling force, air gap is decreased, and the efficiency of the receiver is lowered down.

When a load of 1000 gr. w. is applied to a diaphragm formed of titanium sheet without forced aging, the deformation is produced, as time elapses, as shown by the curve I in Fig. 3. On the other hand, the deformation 30 produced by applying a load of 1000 gr. w. to a diaphragm formed of titanium sheet, to which heat treatment is made for 10 hours at the temperature of 200° C., is shown by the curve II in Fig. 3. As shown in Fig. 3, the deformation of the diaphragm to which heat treatment is applied does not exceed 3 microns, and the deformation speed after 100 hours is very small. Therefore, the efficiency of the telephone receivers in which a heat-treated diaphragm is used scarcely varies by use.

The higher the temperature for heat treatment is, the shorter the time required for heat treatment is. However, since titanium begins to recrystallize and oxidize at the temperature of about 400° C., it is necessary to make the temperature for heat treatment as under 400° C. The temperature at which the strain aging occurs is near to the room temperature. However, it takes much time before the effect of heat treatment is produced, if a temperature below 100° C. is used, and this is improper for actual practice. It is, therefore, desirable to have the heat treatment temperature within the sphere of 100° C.—400° C.

We claim:

1. A titanium diaphragm for acoustic apparatus, characterized by a diaphragm formed from a titanium sheet and having a relatively low stabilized resonant frequency abruptly changed from a relatively high resonant frequency by a heat treatment applied thereto at a temperature of approximately 200° C., which is above the starting temperature of strain aging of titanium and below the starting temperature of the recrystallization of titanium.

5 2. A diaphragm as in claim 1, in which the low stabilized resonant frequency was abruptly affected by a heat treatment made for more than one hour.

65 3. The method of producing a frequency stable titanium diaphragm for acoustic apparatus comprising the steps of forming the diaphragm from a titanium sheet providing a relatively high resonant frequency characteristic in the diaphragm, heating this formed diaphragm to a temperature above the starting temperature of strain aging of titanium and below the starting temperature of the recrystallization of titanium to abruptly lower and stabilize the resonant frequency of the formed diaphragm.

4. The method of producing the diaphragm of claim 3 characterized in that the step of heating is applied for a period of more than one hour.

5. The method of producing the diaphragm of claim 3 characterized in that the step of heating is carried on 5 between the temperatures of 100° C. and 400° C.

6. The method of producing the diaphragm of claim 3 characterized in that the step of heating is carried on at a temperature of approximately 200° C.

7. The method of producing the diaphragm of claim 6 characterized in that the step of heating is applied for a 10 period of ten hours.

References Cited in the file of this patent

UNITED STATES PATENTS

1,204,096 Waller ----- Nov. 7, 1916

OTHER REFERENCES

Titanium and Its Alloys, Materials and Methods, May 1952, page 131.

Kiessel et al.: Journal of Metals, v. 5, sec. 2, February 1953, pages 331-338.